

1

3,208,944

## STABILIZATION OF LUBRICANTS

Henryk A. Cyba, Chicago, Ill., assigner to Universal Oil Products Company, Des Plaines, Ill., a corporation of Delaware  
No Drawing. Filed Nov. 19, 1962, Ser. No. 238,772  
9 Claims. (Cl. 252—51.5)

This is a continuation-in-part of my copending application Serial No. 48,814, filed August 11, 1960, now Patent 3,093,586, issued June 11, 1963, which, in turn, is a continuation-in-part of application Serial No. 826,408, filed July 13, 1959, now Patent 3,078,230, issued February 19, 1963, and relates to the stabilization of lubricants and, more particularly, to a synergistic inhibitor composition and to the use thereof as an additive in lubricants.

In recent years, stringent requirements for lubricants in certain applications have resulted in the availability of a new class of lubricants referred to in the art as synthetic lubricants. These lubricants do not necessarily replace petroleum oils in conventional usage, but are designed for special applications where the petroleum oils do not function to a satisfactory degree. These synthetic lubricants have found particular use in winter-grade crankcase oils, turbo-engine oils, aviation instruments, automatic weapons, etc. For example, aircraft gas turbines require oils capable of providing satisfactory lubrication at temperatures ranging as low as —65° F. and as high as 425° F. during use. Temperatures up to 600° F. are encountered for intervals of from one to two hours during shut-down. Petroleum lubricants are unsatisfactory at high altitudes or in the winter season for use in machine guns and automatic cannons which frequently could not be made to fire because of congealed lubricants. Because they are used under such stringent conditions, the synthetic lubricants may undergo undesirable deterioration including, for example, formation of deposits, discoloration, change of viscosity, etc. While the features of the present invention are particularly applicable to the stabilization of synthetic lubricants, it is understood that they also may be used for the stabilization of petroleum lubricants.

The synthetic lubricants are of varied types including aliphatic esters, polyalkylene oxides, silicones, esters of phosphoric and silicic acids, highly fluorine-substituted hydrocarbons, etc. Of the aliphatic esters, di-(2-ethylhexyl)sebacate is being used on a comparatively large commercial scale. Other aliphatic esters include dialkyl azelates, dialkyl suberates, dialkyl pimelates, dialkyl adipates, dialkyl glutarates, etc. Specific examples of these esters include dihexyl azelate, di-(2-ethylhexyl)azelate, di-3,5,5-trimethylhexyl glutarate, di-3,5,5-trimethylpentyl glutarate, di-(2-ethylhexyl)pimelate, di-(2-ethylhexyl)adipate, triamyl tricarballylate, pentaerythritol tetracapronate, dipropylene glycol dipelargonate, 1,5-pentanediol-di-(2-ethylhexanone), etc. The polyalkylene oxides include polyisopropylene oxide, polyisopropylene oxide diether, polyisopropylene oxide dicester, etc. The silicones include methyl silicone, methylphenyl silicone, etc., and the silicates include, for example, tetraisooctyl silicate, diphenyl di-n-dodecyl silane, octadecyl tri-n-decyl silane, polysilylmethylenes, silophenylene, various silane mixtures, silicone-ester blends, etc. The highly fluorinated hydrocarbons include fluorinated oil, perfluorohydrocarbons, etc.

Additional synthetic lubricating oils include (1) neopentyl glycol esters in which the ester group contains from 3 to 12 carbon atoms or more, and particularly neopentyl glycol propionates, neopentyl glycol butyrate, neop-

2

pentyl glycol caproates, neopentyl glycol caprylates, neopentyl glycol pelargonates, etc., (2) trimethylol alkanes such as trimethylol ethane, trimethylol propane, trimethylol butane, trimethylol pentane, trimethylol hexane, trimethylol heptane, trimethylol octane, trimethylol decane, trimethylol undecane, trimethylol dodecane, etc., as well as the esters thereof and particularly triesters in which the ester portions each contain from 3 to 12 carbon atoms and may be selected from those hereinbefore specifically set forth in connection with the discussion of the neopentyl glycol esters, and (3) tricresylphosphate, trioctylphosphate, trinonylphosphate, tridecylphosphate, as well as mixed aryl and alkyl phosphates, etc.

The lubricating oils of petroleum origin include those referred to as motor lubricating oil, railroad type lubricating oil, marine oil, transformer oil, turbine oil, transmission oil, differential oil, diesel lubricating oil, gear oil, cutting oil, rolling oil, cylinder oil, hydraulic oil, slushing oil, specialty products oil, etc.

The present invention also is applicable to the stabilization of greases made by compositing metallic soaps with the synthetic lubricating oils described above and are referred to herein as synthetic greases. These metal base synthetic greases may be further classified as lithium base synthetic grease, sodium base synthetic grease, calcium base synthetic grease, barium base synthetic grease, strontium base synthetic grease, aluminum base synthetic grease, barium complex greases, calcium complex greases, sodium-calcium greases, lithium-12-hydroxy stearate greases, lithium-calcium greases, calcium-lead greases, etc. These greases are solid or semi-solid gels and, in general, are prepared by the addition to the synthetic lubricating oil of hydrocarbon-soluble metal soaps or salts of higher fatty acids as, for example, lithium stearate, calcium stearate, aluminum naphthenate, etc. The grease may contain thickening agents such as silica, carbon black, talc, organic modified Bentonite, etc., polyacrylates, amides, polyamides, aluminum imides, phthalocyanines, oxanilides, complex aromatic imides and amides, hydantoin derivatives, benzidine dyes, aryl ureas, methyl N-n-octadecyl terephthalamate, etc. Another type of grease is prepared from oxidized petroleum wax, to which the saponifiable base is combined with the proper amount of the desired saponifying agent, and the resultant mixture processed to produce a grease. Other types of greases in which the features of the present invention are usable include petroleum grease, whale grease, wool grease, etc., and those made from inedible fats, tallow, butcher's waste, etc.

It is general practice to incorporate an anti-oxidant in synthetic lubricants in order to improve the stability thereof. Research continues to search for even better inhibitors in order to further improve the synthetic lubricants and permit their use for longer periods of time in present applications, as well as to permit their use under even more severe conditions as, for example, in the engines of the future which are being developed to operate at peak efficiency at high altitudes. It is important that the synthetic lubricant under these conditions is stable, retains its lubricity properties, does not develop deposit formation, retains its desirable viscosity, etc.

It now has been found that a synergistic composition of both an antioxidant and certain nitrogen-containing polymers impart to the synthetic lubricant a considerably improved stability, much greater than obtained through the use of the antioxidants alone. In fact, this synergistic effect is surprising because the polymers themselves do not improve the stability of the synthetic lubricant to

any substantial extent. Normally it would be predicted that this mixture would not be any better than the antioxidant alone. Accordingly, it is surprising that these great improvements in the stability of the lubricant are obtained through the use of the novel inhibitor mixture of the present invention.

In one embodiment the present invention relates to a method of stabilizing a lubricant which comprises incorporating therein a stabilizing concentration, in a synergistic proportion, of a diaminodiphenyl ether antioxidant and a synergist comprising a polymeric condensation product of an acrylate and an alkylaminoalkyl acrylate.

In a specific embodiment the present invention relates to a method of stabilizing di-(2-ethylhexyl)sebacate which comprises incorporating therein a stabilizing concentration, in a synergistic proportion, of 2,4'-di-sec-butyl-diaminodiphenyl ether and a polymeric condensation product of lauryl methacrylate and beta-diethylaminoethyl methacrylate.

In another specific embodiment the present invention relates to a method of stabilizing lithium base grease which comprises incorporating therein a stabilizing concentration, in a synergistic proportion, of 4,4'-di-sec-butyl-diaminodiphenyl ether and a polymeric condensation product of n-octyl methacrylate and beta-diethylaminoethyl methacrylate.

Any suitable diaminodiphenyl ether is used as the antioxidant component of the inhibitor composition. Preferred diaminodiphenyl ethers include N,N'-diisopropyl-diaminodiphenyl ether, N,N'-di-sec-butyl-diaminodiphenyl ether, N,N'-di-sec-amyl-diaminodiphenyl ether, N,N'-di-sec-hexyl-diaminodiphenyl ether, N,N'-di-sec-heptyl-diaminodiphenyl ether, N,N'-di-sec-octyl-diaminodiphenyl ether, N,N'-di-sec-nonyl-diaminodiphenyl ether, N,N'-di-sec-decyl-diaminodiphenyl ether, N,N'-di-sec-undecyl-diaminodiphenyl ether, N,N'-di-sec-dodecyl-diaminodiphenyl ether, N,N'-di-sec-tridecyl-diaminodiphenyl ether, N,N'-di-sec-tetradecyl-diaminodiphenyl ether, etc. Other antioxidants include N,N'-di-cyclohexyl diaminodiphenyl ether and alkylated derivatives thereof. The amino groups are preferably in the 4,4' and/or 2,4'-positions.

In another embodiment the diaminodiphenyl ether antioxidant is an aminophenyl alkoxyphenyl ether. Illustrative preferred antioxidants in this embodiment include 4-methoxyphenyl-4'-aminophenyl ether, 4-methoxyphenyl-4'-N-methyl-aminophenyl ether, 4-methoxyphenyl-4'-N-ethyl-aminophenyl ether, 4-methoxyphenyl-4'-N-isopropyl-aminophenyl ether, 4-methoxyphenyl-4'-N-sec-butyl-aminophenyl ether, 4-methoxyphenyl-4'-N-sec-amyl-aminophenyl ether, 4-methoxyphenyl-4'-cyclohexyl-aminophenyl ether, etc., 4-methoxyphenyl-2'-aminophenyl ether, 4-methoxyphenyl-2'-N-methyl-aminophenyl ether, 4-methoxyphenyl-2'-N-ethyl-aminophenyl ether, 4-methoxyphenyl-2'-N-isopropyl-aminophenyl ether, 4-methoxyphenyl-2'-N-sec-butyl-aminophenyl ether, 4-methoxyphenyl-2'-N-sec-amyl-aminophenyl ether, 4-methoxyphenyl-2'-N-cyclohexyl-aminophenyl ether, etc., 2-methoxyphenyl-4'-aminophenyl ether, 2-methoxyphenyl-4'-N-methyl-aminophenyl ether, 2-methoxyphenyl-4'-ethyl-aminophenyl ether, 2-methoxyphenyl-4'-N-isopropyl-aminophenyl ether, 2-methoxyphenyl-4'-N-sec-butyl-aminophenyl ether, 2-methoxyphenyl-4'-N-sec-amyl-aminophenyl ether, 2-methoxyphenyl-4'-N-cyclohexyl-aminophenyl ether, etc.

Illustrative compounds containing two alkoxy groups include 2,6-dimethoxyphenyl-4'-aminophenyl ether, 2,4-dimethoxyphenyl-4'-aminophenyl ether, 3,4-dimethoxyphenyl-4'-aminophenyl ether, 2,4-dimethoxyphenyl-2'-aminophenyl ether, 3,4-dimethoxyphenyl-2'-aminophenyl ether, etc., and similar compounds in which a hydrocarbon substituent is attached to the nitrogen atom, the hydrocarbon substituent preferably being selected from those hereinbefore set forth. Illustrative examples containing hydrocarbon substituents attached directly to the nucleus of one or both of the phenyl rings include 2-methoxy-4-methylphenyl-4'-aminophenyl ether, 4-methox-

y-2-methylphenyl-4'-aminophenyl ether, 2,6-dimethoxy-4-methylphenyl-4'-aminophenyl ether, 2-methyl-4-methoxyphenyl-2'-aminophenyl ether, 2-methyl-4,6-dimethoxyphenyl-2'-aminophenyl ether, etc. It is understood that other hydrocarbon groups and particularly those hereinbefore set forth may be substituted for the methyl group and also that the nitrogen atom may contain a hydrocarbon constituent attached thereto, the latter substituent preferably being selected from those hereinbefore set forth.

It is understood that different antioxidants are not necessarily equivalent, but all of them will form a synergistic mixture with the acrylate-alkylaminoalkyl acrylate condensation product and will produce improved benefits over and above those expected from the use of either component separately.

The polymeric condensation product for use in the synergistic mixture is produced by the polymeric condensation of an unsaturated compound having a polymerizable ethylenic linkage and an unsaturated compound having a polymerizable ethylenic linkage and a basic nitrogen. In a preferred embodiment the first-mentioned unsaturated compound is amine free and contains from 8 to 18 carbon atoms in an acyclic chain. Examples of such compounds include saturated and unsaturated long chain esters of unsaturated carboxylic acids such as 2-ethylhexyl acrylate, nonyl acrylate, decyl acrylate, undecyl acrylate, dodecyl acrylate, tridecyl acrylate, tetradecyl acrylate, pentadecyl acrylate, hexadecyl acrylate, heptadecyl acrylate, octadecyl acrylate, etc., and particularly methacrylates including n-octyl methacrylate, n-nonyl methacrylate, 3,5,5-trimethylhexyl methacrylate, n-decyl methacrylate, sec-capryl methacrylate, lauryl methacrylate, dodecyl methacrylate, tridecyl methacrylate, tetradecyl methacrylate, pentadecyl methacrylate, hexadecyl methacrylate, cetyl methacrylate, heptadecyl methacrylate, octadecyl methacrylate, 9-octadecenyl methacrylate, etc.; unsaturated esters of long-chain carboxylic acids such as vinyl laurate, vinyl stearate; long-chain esters of vinylene dicarboxylic acids such as methyl lauryl fumarate; long-chain monoolefins such as the alkyl or acyl substituted styrenes as, for example, dodecyl styrene, and the like. A particularly preferred compound is lauryl methacrylate and more particularly technical lauryl methacrylate which is obtained by esterification of a commercial mixture of long-chain alcohols in the C<sub>10</sub> to C<sub>18</sub> range derived from coconut oil. The technical lauryl methacrylate is available commercially at a lower price and, accordingly, is preferred. A typical technical lauryl methacrylate will contain in the ester portion carbon chain lengths of approximately 3% C<sub>10</sub>, 61% C<sub>12</sub>, 23% C<sub>14</sub>, 11% C<sub>16</sub>, and 2% C<sub>18</sub>.

Examples of the second-mentioned unsaturated compounds (those containing a basic nitrogen) include p-(beta-diethylaminoethyl)-styrene; basic nitrogen-containing heterocycles carrying a polymerizable ethylenically unsaturated substituent such as the vinyl pyridines and the vinyl alkyl pyridines as, for example, 2-vinyl-5-ethyl pyridine; esters of basic amino alcohols with unsaturated carboxylic acids such as the alkyl and cycloalkyl substituted aminoalkyl and aminocycloalkyl esters of the acrylic and alkacrylic acids as, for example, beta-methaminoethyl acrylate, beta-diethylaminoethyl methacrylate, 4-diethylaminoethyl methacrylate, beta-beta-didodecylaminoethyl acrylate, etc.; unsaturated ethers of basic amino alcohols such as the vinyl ethers of such alcohols as, for example, beta-aminoethyl vinyl ether, beta-diethylaminoethyl vinyl ether, etc.; amides of unsaturated carboxylic acids wherein a basic amino substituent is carried on the amide nitrogen such as N-(beta-dimethylaminoethyl)-acrylamide; polymerizable unsaturated basic amines such as diallylamine, and the like.

The above polymeric condensation product is prepared in any suitable manner and generally by heating the reactants at a temperature of from about 100° to about

175° F. for a period of time ranging from two to forty-eight hours or more, preferably in the presence of a catalyst or initiator such as benzoyl peroxide, tertiary butyl peroxide, azo compounds as alpha, alpha'-azo-diisobutyronitrile, etc. When desired, the polymerization may be effected in the presence of a solvent and particularly aromatic hydrocarbons, including, for example, benzene, toluene, xylene, cumene, decalin, naphtha, etc. In general the condensation is effected using the first-mentioned and the second-mentioned unsaturated compounds in proportions to produce a copolymer containing from about 50% to about 95% and preferably from about 70% to about 90% by weight of the first-mentioned compound and from about 5% to about 50% and preferably from about 10% to about 30% by weight of the second-mentioned compound.

The proportions of antioxidant and synergist may vary over a wide range and thus may range from 0.1 to 4 and preferably from 0.5 to 2 parts by weight of synergist per one part by weight of antioxidant, although in some cases lower or higher proportions may be used. These proportions are based upon the active ingredient exclusive of solvent. While the antioxidant and synergist may be added separately to the lubricant, it generally is preferred to form a suitable mixture of the antioxidant and synergist and add the mixture to the lubricant. When desired, the antioxidant and synergist may be prepared as a solution in a suitable solvent, particularly aromatic hydrocarbons and more particularly an aromatic hydrocarbon as hereinbefore set forth, and marketed or used as a single product. Conveniently, the same solvent is used in the final solution as used in the preparation of one or both of the antioxidant and synergist. The solution may comprise from about 10% to about 90% and preferably from about 25% to about 75% by weight of active ingredient.

The inhibitor composition will be used in the substrate in an amount sufficient to obtain the desired stabilization. This stabilizing concentration will be within the range of from about 0.01% to about 15% and preferably from about 0.1% to about 5% by weight of the lubricant. The inhibitor composition is added to the lubricant in any suitable manner and preferably with intimate mixing in order to obtain distribution of the inhibitor composition in the lubricant. In some cases the inhibitor composition may be added to the lubricant during the manufacture thereof. For example, when used in grease, the inhibitor composition may be added to one or more of the components before final compositing thereof.

It is understood that the inhibitor composition of the present invention may be used along with other additives incorporated in the lubricant. For example, a metal deactivator, dye, viscosity index improver, pourpoint depressant, antifoaming additive, lubricity and extreme pressure additive, antiscuffing additive, antifriction additive, antiwear additive, detergent-dispersant, etc., may be incorporated in the synthetic lubricant. When desired, the inhibitor composition of the present invention may be prepared as a mixture with one or more of these other additives and incorporated in this manner in the lubricant.

The following examples are introduced to illustrate further the novelty and utility of the present invention but not with the intention of unduly limiting the same.

#### EXAMPLE I

The polymeric condensation product is prepared by copolymerizing lauryl methacrylate and diethylaminoethyl methacrylate in concentrations to yield a product having 80% by weight of lauryl methacrylate and 20% by weight of diethylaminoethyl methacrylate. The polymerization is effected by heating the reactants at about 140° F. for about eighteen hours, with vigorous stirring in the presence of benzoyl peroxide catalyst. The product is recovered as a straw colored, heavy viscous oil of the general properties set forth in Table I.

Table I

|                               |                     |
|-------------------------------|---------------------|
| Viscosity at 210° F., SSU     | 2200.               |
| Density, pounds/gallon        | 7.5.                |
| Color, N.P.A.                 | 1.                  |
| 5 Pour point, ° F.            | -10 to +10.         |
| Flash point (COC), ° F.       | 380.                |
| Fire point (COC), ° F.        | 420.                |
| Total acidity                 | 0.0.                |
| 10 Total base No., mg. KOH/g. | 8.0 (0.14 meq./g.). |
| Ash, weight percent           | 0.00.               |

#### EXAMPLE II

As hereinbefore set forth, the improved results obtained by using the mixture of the present invention are surprising because the polymeric condensation product itself is not an inhibitor. This is shown by the data in the following table, which were obtained in the following manner. The polymeric condensation product was evaluated in diethyl sebacate, marketed under the trade name of "Plexol 201." The evaluation was made in accordance with an Oxygen Stability Test in which a 100 cc. sample of the synthetic lubricating oil is placed in a bath maintained at 400° F. and air is blown therethrough at a rate of 5 liters of air per hour. The sample of synthetic lubricating oil is examined periodically and the time to reach an acid number of 5 is reported. It is apparent that the longer the time required to reach an acid number of 5 the more stable is the sample of synthetic lubricating oil. In other words, it takes longer for the more stable oil to deteriorate.

Table II

| Additive:                                                       | Hours to acid number of 5 |
|-----------------------------------------------------------------|---------------------------|
| None                                                            | 9                         |
| 1% by weight of the polymeric condensation product of Example I | 10                        |

From the above data it will be seen that the polymeric condensation product itself was not effective to extend the time required to reach an acid number of 5.

#### EXAMPLE III

The synergistic mixture of this example is a mixture of 2,4'-di-sec-butyl-diaminodiphenyl ether and the polymeric condensation product of Example I. When evaluated in another sample of the diethyl sebacate described in Example I, the diaminodiphenyl ether, in a concentration of 1% by weight, increases the time to an acid number of 5 from 9 hours to 35 hours. However, the synergistic mixture of 1% by weight of the diaminodiphenyl ether and 1% by weight of the condensation product of Example I increases the time to reach an acid number of 5 to more than 50 hours.

#### EXAMPLE IV

Another advantage of the synergistic mixture of the present invention is that it also considerably reduces sludge and varnish formation as a result of inhibiting deterioration of the lubricating oil during use. The following data reports results in a Chevrolet L-4 test. This test is run using an engine speed of 3150 r.p.m., an engine load of 30 B.H.P., a jacket outlet temperature of 210° F., a jacket inlet temperature of 190° F., an oil temperature of 280° F. and an air fuel ratio of 14.5:1. Regular grade gasoline and Mid-Continent solvent refined S.A.E. 20 type lubricating oil are used. Each run is continued for 36 hours.

The synergistic mixture of this example is 0.5% by weight of a mixture of 70% by weight of 2,4'-di-sec-butyl-diaminodiphenyl ether and 30% by weight of 4,4'-di-sec-butyl-diaminodiphenyl ether and 1% by weight of the polymeric condensation product of Example I.

The following table reports the results of three runs conducted in the manner described above. In the first run (Run A), no additive was incorporated in the lubri-

cating oil. In the second run (Run B), 0.5% by weight of the mixture of 70% by weight of 2,4'-di-sec-butyl-diaminodiphenyl ether and 30% by weight of 4,4'-di-sec-butyl-diaminodiphenyl ether was incorporated in the lubricating oil. In the third run (Run C), a synergistic mixture of 0.5% by weight of the mixture of 70% by weight of 2,4'-di-sec-butyl-diaminodiphenyl ether and 30% by weight of 4,4'-di-sec-butyl-diaminodiphenyl ether and 1% by weight of the polymeric condensation product of Example I was incorporated in the lubricating oil.

Pertinent data of these runs are reported in the following table:

Table III

|                                               | Run A (No Additive)                                                        | Run B (Diaminodiphenyl ether) | Run C (Synergistic mixture) |
|-----------------------------------------------|----------------------------------------------------------------------------|-------------------------------|-----------------------------|
| Total varnish and sludge, gravimetric, grams. | (Run was discontinued after 12 hours due to excessive noise.)<br>At 8 hrs. | 7.289<br>At 36 hrs.           | 1.767<br>At 36 hrs.         |
| Used oil analyses:                            |                                                                            |                               |                             |
| Pentane insolubles, wt. percent               | 0.449                                                                      | 0.786                         | 0.376                       |
| Benzene insolubles, wt. percent               | 0.237                                                                      | 0.541                         | 0.242                       |
| Insoluble resin, wt. percent                  | 0.212                                                                      | 0.245                         | 0.134                       |
| Viscosity, S.S.U. at 400° F.                  | 608                                                                        | 358                           | 354                         |

From the above table, it will be seen that the synergistic mixture served to improve the operation of the engine as compared to the run without inhibitor and to the run made with the diaminodiphenyl ether alone. Of special importance is the considerably lower amount of total varnish and sludge. It will be noted that Run A had to be discontinued after 12 hours. In Run B, the total varnish and sludge was greater than 7 grams, whereas it was less than 2 grams in Run C using the synergistic mixture.

## EXAMPLE V

The synergistic mixture of this example comprised 0.5% by weight of 2,4'-di-sec-butyl-diaminodiphenyl ether and 1% by weight of the polymeric condensation product of Example I.

The results of runs made in the same manner as described in Example IV are reported in the following table:

Table IV

|                                               | Run D (No Additive)                                                       | Run E (Diaminodiphenyl ether) | Run F (Synergistic mixture) |
|-----------------------------------------------|---------------------------------------------------------------------------|-------------------------------|-----------------------------|
| Total varnish and sludge, gravimetric, grams. | (Run was discontinued after 12 hours due to excessive noise)<br>At 8 hrs. | 7.745<br>At 36 hrs.           | 2.029<br>At 36 hrs.         |
| Used oil analyses:                            |                                                                           |                               |                             |
| Pentane insolubles, wt. percent               | 0.449                                                                     | 0.786                         | 0.376                       |
| Benzene insolubles, wt. percent               | 0.237                                                                     | 0.541                         | 0.242                       |
| Insoluble resin, wt. percent                  | 0.212                                                                     | 0.245                         | 0.134                       |
| Viscosity, S.S.U. at 400° F.                  | 608                                                                       | 358                           | 354                         |

Here again, it is seen that the synergistic mixture of the present invention considerably improved the operation of the engine and inhibited deterioration of the lubricating oil during use.

As hereinbefore set forth, the cleanliness of the oil during use is very important and could mean the difference between an additive which would be acceptable and one which would not be acceptable. The cleanliness is evaluated by determining the percent isoctane insolubles, the percent viscosity change and the appearance of the tube after use. The following table reports results made in diethyl sebacate evaluated in the stability test described in Example II in which the determinations were made after 48 hours exposure and the viscosity change was determined at 130° F. In these tests, 2% by weight of the additives were used. These data are reported in the following table:

|    | Additive                                                     | Percent Isoctane Insolubles* | Percent Viscosity Change* | Tube Appearance*                         |
|----|--------------------------------------------------------------|------------------------------|---------------------------|------------------------------------------|
| 20 | 2% by weight of 2,4'-di-sec-butyl-diaminodiphenyl ether.     | 1.53                         | 16                        | Messy, considerable varnish and deposit. |
| 25 | 2% by weight of polymeric condensation product of Example I. | 0.23                         | 165                       | Clean, no varnish, no deposit.           |
| 25 | 2% by weight of each of the above additives.                 | 1.7                          | 4.3                       | Do.                                      |

\*Determined after 48 hours.

Here again, the synergistic effect is clearly demonstrated. It normally would be expected that the percent isoctane insolubles would be an average of the total of those obtained with each additive alone ( $1.53+0.23=10.76$  which, divided by 2, gives an average of 5.38 isoctane insolubles). It will be noted that the percent isoctane insolubles formed when using the mixture amounts to only 1.7%. The same applies to the percent viscosity change which normally would be expected to be about 90% ( $16+165=181$  divided by 2=90). Instead, and surprisingly, the viscosity change is only 4.3% when using the mixture of additives. The same also applies to the appearance of the tube. Certainly, if one of the additives forms varnish and deposits when used alone, it would be expected that a mixture including such additive would likewise do so. However, as shown by the above data, the expected result did not occur but instead the tube was clean.

## EXAMPLE VII

As hereinbefore set forth, a synthetic lubricant being considered for use at high temperature is pentaerythritol ester. The pentaerythritol ester used in this example is available commercially from Hercules Powder Company as "Hercoflex 600" and is stated to be monomeric pentaerythritol ester having an acid number of 0.10 maximum, a saponification number of 410, a refractive index at 20° C. of 1.453 and a specific gravity at 25/25° C. of 0.997.

The evaluations in the pentaerythritol ester are made in substantially the same manner as described in Example II for diethyl sebacate. The synergistic inhibitor mixture of this example is 1% by weight of 4-methoxyphenyl-4'-N-isopropyl-aminophenyl ether and 1% by weight of the polymeric condensation product of Example I.

When evaluated in the pentaerythritol ester in the same manner as described for the diethyl sebacate, except conducted at 500° F. instead of 400° F., the synergistic mixture had a longer time to acid number of 5 than obtained with either component alone. It was compared with a sample of the pentaerythritol ester containing 1% by weight of the 4-methoxyphenyl-4'-N-isopropyl-aminophenyl ether and with a separate sample containing 2% by weight of the polymeric condensation product of Example I. The percent isoctane insolubles was lower for the synergistic mixture than when using either component alone and, of particular importance, is the fact that the

percent viscosity change was 62% as compared to the viscosity change of 134% for the sample of lubricating oil containing the polymeric condensation product.

#### EXAMPLE VIII

Another synthetic lubricating oil consists of esters of trimethylolpropane. A lubricating oil available commercially comprises trimethylolpropane esters having an average molecular weight of about 457 and the ester portions have an average of 7 carbon atoms each. Typical properties of such a lubricating oil, available commercially from the Celanese Corporation of America under the trade name of "Cellutherm," are set forth below.

|                             |        |
|-----------------------------|--------|
| Specific gravity, 60/60° F. | 0.965  |
| Acidity, mg./KOH/g.         | 0.03   |
| Color, ASTM                 | 2      |
| Fire point, COC, °F.        | 520    |
| Flash point, COC, °F.       | 460    |
| Hydrolysis number           | 0.27   |
| Viscosity:                  |        |
| At -65° F., cs.             | 14,900 |
| At 100° F., SSU             | 76.93  |
| At 210° F., SSU             | 37.77  |

The antioxidant, polymeric condensation product and synergistic mixture described in Example VII also were evaluated in the above synthetic lubricating oil. Here again, it is noted that the hours to acid number of 5 were greater for the synergistic mixture than were obtained with either of the components alone and also that the viscosity change was 34% as compared to 47% for the sample of lubricating oil containing the antioxidant alone and 66% for the sample containing the polymeric condensation product alone.

#### EXAMPLE IX

The synergistic inhibitor mixture of this example is 1% by weight of 2,4'-dicyclohexyl-diaminodiphenyl ether and 1% by weight of the polymeric condensation product of Example I.

When evaluated in another sample of the dioctyl sebacate in the same manner as described in Example II, the induction period of the synthetic lubricating oil is increased from 9 to about 64 hours which, it will be noted, is considerably more than the total of 41 hours obtained with the inhibitor alone and the 4 hours obtained with the polymeric condensation product alone.

#### EXAMPLE X

The synergistic inhibitor mixture of this example is 1.5% by weight of 4,4'-dicyclohexyl-diaminodiphenyl ether and 0.75% by weight of the polymeric condensation product formed by n-octyl-methacrylate and diethyl aminoethyl methacrylate.

When evaluated in the pentaerythritol ester hereinbefore described, the synergistic mixture serves to extend the induction period of the lubricating oil from 16 hours to more than 65 hours.

#### EXAMPLE XI

The synergistic mixture of this example is 1% by weight of 2,4'-di-sec-butyl-diaminodiphenyl ether and 0.5% by weight of the condensation product of Example I. It is utilized as an additive in lithium base grease.

The synergistic inhibitor mixture is incorporated in lubricating oil in the concentrations described above and the lubricating oil then is mixed with approximately 8% by weight of lithium stearate. The mixture is heated to about 450° F. with constant agitation. Subsequently the grease is cooled, while agitating, to approximately 250° F. and then is further cooled slowly to room temperature. 70

When evaluated in a bomb charged with oxygen at a temperature of 50° F., the induction period is determined as the time required for a drop of 5 pounds pressure to occur. The synergistic mixture serves to increase the induction period of the grease from 7 hours to over 200 hours.

I claim as my invention:

1. A synergistic inhibitor composition of 1 part by weight of N,N'-di-sec-butyl-diaminodiphenyl ether and from about 0.1 to about 4 parts by weight of the polymeric condensation product, formed at a temperature of from about 100° to about 175° F., of from about 50% to about 95% by weight of lauryl methacrylate and from about 5% to about 50% by weight of beta-diethylaminoethyl methacrylate.

2. A synergistic inhibitor composition of 1 part by weight of N,N'-dicyclohexyl-diaminodiphenyl ether and from about 0.1 to about 4 parts by weight of the polymeric condensation product, formed at a temperature of from about 100° to about 175° F., of from about 50% to about 95% by weight of lauryl methacrylate and from about 5% to about 50% by weight of beta-diethylaminoethyl methacrylate.

3. A synergistic inhibitor composition of 1 part by weight of 4-methoxyphenyl N-isopropylaminophenyl ether and from about 0.1 to about 4 parts by weight of the polymeric condensation product, formed at a temperature of from about 100° to about 175° F., of from about 50% to about 95% by weight of lauryl methacrylate and from about 5% to about 50% by weight of beta-diethylaminoethyl methacrylate.

4. A synergistic inhibitor composition of 1 part by weight of 4-methoxyphenyl N-sec-butylaminophenyl ether and from about 0.1 to about 4 parts by weight of the polymeric condensation product, formed at a temperature of from about 100° to about 175° F., of from about 50% to about 95% by weight of lauryl methacrylate and from about 5% to about 50% by weight of beta-diethylaminoethyl methacrylate.

5. A lubricating composition comprising a major proportion of a lubricant and from about 0.001% to about 5% by weight of the synergistic inhibitor composition of claim 1.

6. A lubricating composition comprising a major proportion of a lubricant and from about 0.001% to about 5% by weight of the synergistic inhibitor composition of claim 2.

7. A lubricating composition comprising a major proportion of a lubricant and from about 0.001% to about 5% by weight of the synergistic inhibitor composition of claim 3.

8. A lubricating composition comprising a major proportion of a lubricant and from about 0.001% to about 5% by weight of the synergistic inhibitor composition of claim 4.

9. A lubricating composition comprising a major proportion of dioctyl sebacate and from about 0.001% to about 5% by weight of the synergistic inhibitor composition of claim 1.

#### References Cited by the Examiner

##### UNITED STATES PATENTS

|           |       |              |            |
|-----------|-------|--------------|------------|
| 2,737,496 | 3/56  | Cathin       | 252—51.5   |
| 2,892,784 | 6/59  | Harle et al. | 252—47.5   |
| 2,910,437 | 10/59 | Symon        | 252—51.5   |
| 2,926,093 | 2/60  | Cyba         | 252—403 X  |
| 2,964,479 | 12/60 | Cyba         | 252—51.5 X |

DANIEL E. WYMAN, Primary Examiner.